

Jan. 16, 1923.

1,442,328.

J. DE LONG.

INSULATING MATERIAL AND PROCESS OF MANUFACTURING SAME.  
FILED SEPT. 29, 1922.



*Julius De Long*

INVENTOR

*Henry D. P. <sup>BY</sup> Knipe* *att* *ATTORNEY*

## UNITED STATES PATENT OFFICE.

JULIUS DE LONG, OF LAKE MAHOPAC, NEW YORK.

## INSULATING MATERIAL AND PROCESS OF MANUFACTURING SAME.

Application filed September 29, 1922. Serial No. 591,362.

*To all whom it may concern:*

Be it known that I, JULIUS DE LONG, a citizen of the United States, residing at Lake Mahopac, in the county of Putnam, 5 State of New York, have invented new and useful Improvements in Insulating Materials and Processes of Manufacturing Same, of which the following is a specification.

My invention relates to improvements in 10 insulating material which are particularly adapted for use in insulating railroad cars, buildings and other structures, and in the process of manufacturing the same; and the other objects of my invention are to produce 15 a new insulating material which can be cheaply and economically manufactured and which will be fireproof in its character.

Reference is hereby made to the following 20 pending applications by the applicant relating to the same or kindred subject matter, namely: Serial No. 432,649, Serial No. 517,923 and Serial No. 556,579.

Figure 1 is a perspective view of my insulating material with the layers of the material used partly broken away. Fig. 2 is an enlarged sectional view on the line *x x* of Figure 1. In the drawings, 1 indicates the woven fabric; 2 the bats of asbestos fibre, and 3 the covering of asbestos paper.

Heretofore, fireproof insulating material has been made from asbestos fibre, but in 30 this type of insulating material the fibres were always secured together by glue or other adhesive material, which tended to 35 close and fill the air spaces between the fibres and thereby greatly decrease the insulating value of the insulating material. Material so formed is liable to disintegrate and fall apart when wet and therefore is 40 undesirable for many purposes for which insulating material is used.

I have found that I can make a strong, durable and substantially fireproof insulating material by the following process:

I run asbestos fibre through a picker until 45 it has been finely divided and then form the asbestos fibre into a bat by running it through a carding machine. I lay a bat so formed upon a strip of fireproofed burlap 50 or other suitable, non-inflammable woven fabric possessing the desired strength, and run the bat and burlap through a needle punching loom, the needles of such loom forcing the finely divided asbestos fibre 55 through the woven fabric and interlocking the fibres of asbestos with each other and

thereby firmly securing the bat to the woven fabric, the fibres being of such small diameter that they will not be broken by this step in my process. When this operation is 60 completed I turn the product over and place another similarly formed bat upon the exposed surface of the woven fabric and again run the material through a punching needle loom, with the result that the fibres 65 of asbestos in the upper bat are interlocked and the fibres of the upper bat are driven through the woven fabric and more or less interlocked with the asbestos fibres on the opposite side and with the woven fabric. 70

This produces a strong, durable felt which 75 is a better nonconductor of heat than the material heretofore used, and is at the same time essentially fireproof. Where burlap is used I treat the burlap with a solution which 80 renders it flame proof. Where a rigid material is required I apply adhesive material to the surface of asbestos paper which I apply under pressure to one or both of the outer surfaces of the felt formed as above 85 stated. Where asbestos is so applied and particularly where it is applied to both sides of the felt, the insulating value is increased because of the dead air trapped between the sheets of asbestos paper. Where asbestos 90 paper is applied to both sides of the felt the finished product possesses sufficient rigidity and strength to be easily handled and applied.

Having described my invention, I claim: 90

1. The process of manufacturing insulating material which consists of finely dividing asbestos fibre by running it through a picker; second, running the finely divided asbestos fibre through a carding machine and forming 95 it into a bat; third, laying the bat so formed upon a strip of woven fabric and running the bat and fabric through a punching needle loom; fourth, placing a similarly formed bat of asbestos fibre on the 100 exposed surface of the woven fabric and again running the thus assembled bats and woven fabric through a punching needle loom; and fifth, applying adhesive material to the surface of asbestos paper and applying such paper to the outer surfaces of the 105 felt so formed.

2. The process of manufacturing insulating material which consists of finely dividing asbestos fibre by running it through a 110 picker; second, running the finely divided asbestos fibre through a carding machine

and forming it into a bat; third, laying the bat so formed upon a strip of non-inflammable woven fabric and running the bat and fabric through a punching needle loom; 5 fourth, placing a similarly formed bat of asbestos fibre on the exposed surface of the woven fabric and again running the thus assembled bats and woven fabric through a punching needle loom; and fifth, applying 10 adhesive material to the surface of asbestos paper and applying such paper to the outer surfaces of the felt so formed.

3. An insulating material comprising in combination woven fabric, bats of finely divided asbestos fibre on each side of such woven fabric, the asbestos fibres in each bat being interlocked with each other, with the woven fabric and with the asbestos fibres on the opposite side of such woven 15 fabric.

4. An insulating material comprising in combination non-inflammable woven fabric, bats of finely divided asbestos fibre on each side of such non-inflammable woven 20 fabric, the asbestos fibres in each bat being 25

interlocked with each other, with the non-inflammable woven fabric and with the asbestos fibres on the opposite side of such non-inflammable woven fabric.

5. An insulating material comprising in 30 combination woven fabric, bats of finely divided asbestos fibre on each side of such woven fabric, the asbestos fibres in each bat being interlocked with each other, with the woven fabric, with the asbestos fibres on the 35 opposite side of such woven fabric and asbestos covering on each side thereof and secured thereto by adhesive material.

6. An insulating material comprising in combination non-inflammable woven fabric, 40 bats of finely divided asbestos fibre on each side of such non-inflammable woven fabric, the asbestos fibres in each bat being interlocked with each other, with the non-inflammable woven fabric, with the asbestos fibres on the opposite side of such non-inflammable woven fabric and asbestos covering on each side thereof and secured 45 thereto by adhesive material.

JULIUS DE LONG.